

# United States Patent Office

2,781,306

Patented Feb. 12, 1957

1

2,781,306

## ELECTRODEPOSITION OF NICKEL

Henry Brown, Huntington Woods, Mich., assignor to The Udylite Research Corporation, Detroit, Mich., a corporation of Michigan

No Drawing. Application April 27, 1956,  
Serial No. 580,990

4 Claims. (Cl. 204—49)

This invention relates to the electrodeposition of nickel from an aqueous acidic bath.

One object of this invention is to decrease the grain size and increase the luster of the nickel deposit.

A second and major object is the electrodeposition of brilliant, highly lustrous, ductile nickel plate.

It has been found that these objects can be accomplished by the use of certain organic compounds in the aqueous acidic nickel baths.

The first object can be accomplished by the addition to the Watt's type of nickel bath or its modifications, of certain organic compounds which contain unsaturated linkages, such as the aldehydic (and ketonic carbonyl), the olefinic type of unsaturated bond, double or triple, and the unsaturated carbon to nitrogen bond, double or triple, i. e.



Compounds in the bath containing such groups cause the nickel plate to be very fine grained (even though cloudy and milky in appearance) and show marked increasing lustre with continued plating.

However, not all unsaturated linkages produce the desired effects, for example, unsaturated bonds not connected to carbon, for example,  $\text{N}=\text{O}$ ,  $\text{N}=\text{N}$ . Also the unsaturated bonds carbon to carbon, carbon to oxygen, or carbon to nitrogen, where an  $-\text{OH}$ , or  $-\text{NH}_2$ , or  $-\text{NH}-$  group is also attached to the carbon atom carrying the unsaturated bond, for example:



It was further found that the second object, the production of brilliant highly lustrous ductile nickel plate, could be accomplished by the use in conjunction with the active unsaturated groups (1), another, different functional group, namely the methylene sulfone group



as exemplified by aryl sulfonamides and sulfonimides, or aryl sulfonic acids. Compounds with either group alone in the bath give no obvious indication of the remarkably different and enhanced result which occurs when both groups are present.

The first object mentioned above can also be accomplished by the addition to the Watt's type of nickel bath or its modifications of certain amides carrying an unsaturated olefinic group. The presence of these particular amides, which are more specifically illustrated by the compounds set forth in Table III, may be designated generally by Formula A

## FORMULA A



where  $\text{R}_1$  and  $\text{R}_2$  are selected from the group consisting of hydrogen, acetyl, chlorine, bromine, methyl, methyl

2

carboxy, carbonyl, carboxy and aldehydo, phenyl and furyl and the chloro, bromo, acetyl, methyl, carboxy, amino, methoxy, ethoxy, dioxymethylene, carbonyl amido, hydroxy and ethyl substitution products of phenyl and furyl;  $\text{R}_3$  and  $\text{R}_4$  are selected from the group consisting of hydrogen, methyl, methylene, methylol, formyl, acetyl, amino, amido, imido, carboxy, carbonyl, benzoyl and nicotinoyl radicals. The types of compounds which are encompassed by Formula A are illustrated in the compounds designated A, B, C and D.

## COMPOUND A

When  $\text{R}_1$ ,  $\text{R}_2$ ,  $\text{R}_3$  and  $\text{R}_4$  are hydrogen, we have



## COMPOUND B

When  $\text{R}_1$  is phenyl,  $\text{R}_2$ ,  $\text{R}_3$  and  $\text{R}_4$  are hydrogen, we have



## COMPOUND C

Where  $\text{R}_1$  is methyl carboxy,  $\text{R}_2$ ,  $\text{R}_3$  and  $\text{R}_4$  are hydrogen, we have



Monomethyl maleic acid monoamide (methyl ester of maleamic acid)

## COMPOUND D

When  $\text{R}_1$  is carbonyl,  $\text{R}_2$  and  $\text{R}_3$  are chlorine and  $\text{R}_4$  is hydrogen, we have



## Mucochloric acid amide

The presence of the compounds represented by Formula A in the bath causes the nickel plate which is electro-deposited therefrom to be very fine-grained (even though cloudy and milky in appearance), and to show marked increasing luster with continued plating.

It was further found that the second object, the production of brilliant, highly lustrous, ductile nickel plate, could be accomplished by the use in conjunction with the compounds represented by Formula A, of a material containing another and different functional group, namely, the unsaturated methylene sulfone group



as exemplified by benzene sulfonamides and sulfonimides. The presence of a compound represented by Formula A alone in a Watt's type nickel bath, or the presence of a material containing the unsaturated methylene sulfone group alone, gives no obvious indication of the remarkably different and enhanced result which occurs when both materials are concurrently present.

While the simpler aryl sulfonamides and some of the aryl sulfonic acids produce bright and mirror-like deposits on buffed metals such as buffed brass, they fail to accomplish the same result on steel polished, for example, with 200 emery or on top of matte (but unburnt) copper plate.

of 0.0003"-0.0005" thickness, and yield in these cases plate of dull and grey appearance.

The compounds carrying the active unsaturated groups (olefinic, aldehydic, etc.) while giving a different type of plate than that produced by the aryl sulfones, nevertheless, give at best a cloudy plate on either buffed or matte metal. Their rate of improvement of luster of the base metal is, however, faster than that produced by aryl sulfonamides or aryl sulfonic acids.

If, however, these two different groups are used together, a brilliant mirror-like deposit can be obtained even on the matte copper deposit. The result is very striking from a comparison of the results obtained with either group alone in the bath. This is best illustrated by an example.

If furfural is added to a Watt's bath in the concentration of about 0.7 g./l., a brittle, poorly adherent, fine-grained, cloudy deposit is obtained and seems to be covered with an iridescent film which stains easily. On the addition of 2 g./l. of an aryl sulfone, for example, o-benzoyl sulfimide, a very brilliant, ductile, adherent plate is obtained. Thus not only has the tolerance of the bath been remarkably increased to larger concentrations of the furfural, but there has resulted a plate of striking brilliance.

Furthermore, it is found that with continued plating, the furfural is depleted more slowly in the presence of the aryl sulfone. On analysis of the plates for carbon in the case of furfural alone in a bath containing 250 g./l. of  $\text{NiSO}_4 \cdot 7\text{H}_2\text{O}$ , 60 g./l. of  $\text{NiCl}_2 \cdot 6\text{H}_2\text{O}$ , and 40 g./l. of  $\text{H}_3\text{BO}_3$ , and in the case of the same concentration of furfural used together with 2 g./l. of o-benzoyl sulfimide, it is found that about twice as much carbon is present in the plate with furfural alone (i. e. about 0.28% compared to about 0.17%); the plates were run at the same current density, 30 amps./sq. ft. average.

Mixing any two brighteners in the bath will not give rise to a plate of remarkable brilliance, for example, in mixing an active aldehyde with zinc or cadmium in their employable concentrations. Instead, there is practically no improvement in brightness, but an increase in dull areas and a definite loss of ductility and bond, that is, the latter two types of materials act similarly though not identically in the bath. The active unsaturated compounds, such as furfural, crotonaldehyde, diallylamine, allyl alcohol, have in general the characteristic of producing marked changes in the appearance and character of the plate with increasing concentrations of the unsaturated compounds. As their concentration is increased, the plating of nickel in the very low current densities is practically stopped and with further increase in concentration, streaked, peeled, brittle plate results. The aryl sulfones in general do not have critical concentrations, and they produce practically no further results after their optimum concentration is reached, i. e., they do not produce peeled, streaked plate at any concentration and the baths always plate more easily in the low current density areas than the plain nickel bath. This phenomenon, as well as their life in the bath (which differs extremely), indicates that there is a different rate of reduction of these two types of compounds at the nickel cathode with respect to the nickel ion. In the case of the active unsaturated compounds (olefinic, aldehydic, etc.) there is preferential reduction of the unsaturated compound with respect to the nickel ion, whereas with the aryl sulfones, the nickel ion is reduced preferentially. Thus the effect of the aryl sulfones in the nickel bath on the plating out of small percentages of other ions more easily reduced than the nickel, i. e.  $\text{Cu}^{++}$ ,  $\text{Zn}^{++}$ ,  $\text{Cd}^{++}$ , etc. is also more readily understood. The variation of the reduction with the variation of the cathode potentials between adjacent high and low points will account for the rate of brightening, or "smoothening out" effect, etc. of the various addition agents.

The uniqueness of the aryl sulfones, or broadly the



compounds, seems to be mainly tied up with the rate of reduction of the positive valent sulfur compound to negative valent sulfur compound, and the mechanism of its deposition. The fact that with  $\alpha$ -naphthalene sulfonamide as the only organic compound in the bath, not only is the odor of naphthalene apparent at the cathode during the plating, but the analysis of the plate shows the presence of carbon as well as sulfur, which indicates that the mechanism of the reduction is not of the simplest form.

It is not the sulfone group alone that is responsible for the effect of the aryl sulfones because the saturated alkyl sulfones are not nearly as effective as the aryl sulfones.

Certain substituting groups on the ring detract from the beneficial effect of the



group, i. e., hydroxy groups on the ring, nitro groups, and too many alkyl groups on the ring which introduces insolubility and colloidal nature.

The benzene and toluene sulfonamides and ortho benzoyl sulfimide are more effective than aryl monosulfonic acids, especially of the benzene series, nevertheless the latter, even though they may not produce bright plate on buffed metals, will give brilliant ductile plate when used in combination with the active unsaturated compounds.

The various compounds which carry one or more active unsaturated groups or combinations differ greatly in their degree of effectiveness in a bath when used alone or in conjunction with the aryl sulfone compounds. The compounds which give the most beneficial effects and are the least critical when used alone are in general not the ones that are the most effective when used with the aryl sulfones.

The effectiveness of the unsaturated compounds is greatly dependent on the type and number of unsaturated groups, on their positions in the molecule, and the presence of other groups. For example, the allyl group is much more effective than the beta-methyl allyl. The allyl group is as effective or even more effective than the aldehydic carbonyl.

In the discussion below of the organic compounds containing unsaturated linkages, it is understood that the description relates to these compounds when used with the aryl sulfones in an acid nickel plating bath.

*Olefinic unsaturated compounds.*—Unsaturated alcohols are not as effective as unsaturated aldehydes or unsaturated ketones, which is to be expected from the fact that the saturated alcohols have no effect in the bath when used in the same concentrations. Allyl alcohol is superior to butyraldehyde and also to furfuryl alcohol.

The unsaturated amines are very effective. The three allyl amines, tri-, di-, and mono-allyl amine are the best of the unsaturated amines. The saturated aliphatic amines, on the other hand, are either ineffective or harmful. The unsaturated amides, particularly allyl urea, are very effective and when used alone in the bath, somewhat less critical than the unsaturated amines. The saturated ureas, such as propyl or butyl urea or urea itself have no effect in similar or larger concentrations.

*Other unsaturated compounds.*—The triple bond  $-\text{C}\equiv\text{C}-$  is exceedingly active and only traces of compounds carrying it, such as dimethylethynyl carbinol, can be used even with the aryl sulfones. The aliphatic  $-\text{C}\equiv\text{N}$  compounds such as propionitrile are also exceedingly active and the slightest excess prevents plating at very low current densities and causes highly streaked, brittle, non-adherent plate. The cyano aryl compounds such as cyanobenzoic acid, cyano-benzene sulfonic acid are much less active and do not show the critical effects that the aliphatic do, thus showing again how the properties of even the most active of the unsaturated groups may

be altered by various substitutions to give the desired amount or degree of effect. Furthermore, in the same way, the double bond



is not as critical as the  $-\text{C}\equiv\text{C}-$ , also the



group is not as critical as the  $-\text{C}\equiv\text{N}$ . For example, the compounds: pyridine, quinoline, phenosafranine, "Nitron" (1,4 diphenyl-endanilo-triazoline), etc have the



linkage (aryl or alkyl) and give good results with the aryl sulfones. Imidazole, however, is harmful because an NH group is attached to the carbon of the  $\text{C}=\text{C}$  and  $\text{C}=\text{N}$  bonds. The



linkage is so much more active than the



and



linkages that it produces the desirable effects even when the entire



group is in a ring, as in pyridine, phenosafranine, etc. whereas the



and



groups are not effective when part of an aromatic ring. In fact the compounds carrying the



group (wherein the latter is in a ring and attached by its carbon to another carbon or a tertiary nitrogen) can be used in very small concentrations together with an aryl sulfone to give a brilliant plate, and moreover depletes at a slower rate than do the active olefinic compounds as carbon analysis of their plates also shows.

The concentration of a compound represented by Formula A or a mixture thereof which may be advantageously employed is not critical in any concentration up to saturation, and may be used at concentrations between about 0.1 to about 2.0 grams/liter, the preferred concentration being .6-1.2 grams/liter.

In keeping with their chemical activity, the higher the temperature of the bath, the more active are the unsaturated groups in the bath and smaller concentrations of compounds carrying them must be used. Furthermore, they function best at the higher pH values of the nickel bath, that is, 3.0 to 5.2, and their effectiveness in most cases drops rather suddenly when the pH is lowered past a certain value (in general, at a pH below 3.0 or 2.5, depending on the type of unsaturated compound and on the temperature). The lower the temperature, the higher are the pH values that should be used, and conversely.

The best cathode film buffer is boric acid and it is important to keep its concentration high (over 30 grams/liter), especially in the warm baths. Other buffers may be used in small amounts (1 to 5 grams/liter) with the boric acid with beneficial effects, such as formic, citric, fluoboric acids, etc., but they are not recommended to be used alone.

In the use of a compound represented by Formula A alone in the bath, or in the presence of the aryl sulfones, 75

ammonium salts should be kept at a minimum. A concentration of zinc and copper ions in the bath should also be kept as low as possible. This is especially desirable where the concentration of aryl sulfones are low in the bath or the latter compounds are absent.

The baths may be operated at pH values ranging from 2.0 to 5.5 and temperatures ranging from 20° C. to 70° C. and the preferred current density ranges may be from 5 to 150 amps./sq. ft., depending on the agitation, the temperature of the bath and the concentration and the type of nickel salts. The benzene sulfonamides and sulfonimides may be used effectively in concentrations of from 0.05 gram/liter to saturation. Some of the baths are remarkably free from pitting without the use of auxiliary surface-active materials. This is especially true where the baths are kept clean and free from excessive contamination. Otherwise a straight chain, alkyl benzene sulfonate or a wetting agent such as lauryl alcohol sulphate or iso-octyl alcohol sulphate is desirable.

20 In Table I are listed preferred bath compositions.

Table I

|         | NiSO <sub>4</sub> .<br>6H <sub>2</sub> O, g./l. | NiCl <sub>2</sub> .<br>6H <sub>2</sub> O, g./l. | H <sub>3</sub> BO <sub>3</sub> , g./l. | Ni(BF <sub>4</sub> ) <sub>2</sub> , g./l. | Temp.<br>(° C.) | Opti-<br>mum pH |
|---------|-------------------------------------------------|-------------------------------------------------|----------------------------------------|-------------------------------------------|-----------------|-----------------|
| 25      | 250-300                                         | 35-75                                           | 35-40                                  | -----                                     | 40-65           | 2.5-4.5         |
|         | -----                                           | 100-300                                         | 35-40                                  | -----                                     | 40-65           | 2.5-4.5         |
| 75-100  | 200-250                                         | 35-40                                           | -----                                  | -----                                     | 40-65           | 2.5-4.5         |
| 200-250 | 30-60                                           | 35-40                                           | 7-15                                   | 40-50                                     | 2.8-5.0         | 2.8-5.0         |
| 30      | -----                                           | 0-35                                            | 0-40                                   | 150-300                                   | 40-50           | 2.8-5.0         |

In the case of the very active unsaturated compounds and specifically dimethylethynyl carbinol, trace quantities as little as 0.001 to 0.01 gram/liter give optimum results 35 with benzene sulfonamides and benzene sulfonimides.

In Table II are listed representative examples of organic sulfonamides, sulfonimides and sulfonic acids which may be employed in conjunction with the addition agents of Table III.

Table II

| Sulfur-containing brighteners:                    | Optimum conc.<br>grams/liter |
|---------------------------------------------------|------------------------------|
| 1. Benzene sulfonamide                            | 0.1-3                        |
| 2. Toluene sulfonamides (o- and p-)               | 0.1-2                        |
| 3. o-Benzoyl sulfimide                            | 0.1-2                        |
| 4. N-benzoyl benzene sulfonimide                  | 0.1-1                        |
| 5. p-Toluene sulfonchloramide                     | 0.1-1                        |
| 6. p-Brom benzene sulfonamide                     | 0.1-1                        |
| 7. 6-chlor o-benzoyl sulfimide                    | 0.1-1                        |
| 8. m-Aldehydo benzene sulfonamide                 | 0.1-1                        |
| 9. Sulfomethyl benzene sulfonamide                | 0.1-6                        |
| 10. Benzene sulfonamide m-carboxylic amide        | 0.1-3                        |
| 11. 7-aldehydo o-benzoyl sulfimide                | 0.1-3                        |
| 12. N-acetyl benzene sulfonimide                  | 0.1-2                        |
| 13. Methoxy benzene sulfonamides                  | 0.1-1                        |
| 14. Hydroxymethyl benzene sulfonamide             | 0.1-2                        |
| 15. Vinyl sulfonamide                             | 4-12                         |
| 16. Allyl sulfonamide                             | 4-12                         |
| 17. Benzene sulfonic acids (mono-, di-, and tri-) | 1-15                         |
| 18. p-Brom benzene sulfonic acid                  | 3-6                          |
| 19. Benzaldehyde sulfonic acids (o, m, p)         | 2-6                          |
| 20. Diphenyl sulfone sulfonic acid                | 1-8                          |
| 21. Naphthalene sulfonic acids (mono-, di-, tri-) | 1-8                          |
| 22. Benzene sulfohydroxamic acid                  | 1-5                          |
| 23. p-Chlor benzene sulfonic acid                 | 1-15                         |
| 24. Diphenyl sulfonic acid                        | 1-5                          |
| 25. m-Diphenyl benzene sulfonic acid              | 1-4                          |
| 26. 2-chloro - 5 - sulfobenzaldehyde              | 1-5                          |
| 27. m-Benzene disulfonamide                       | 0.5-1                        |
| 28. Allyl sulfonic acid                           | 4-12                         |
| 29. Cinnamyl sulfonic acid                        | 0.1-8                        |
| 30. Cinnamyl sulfonamide                          | 0.1-3                        |

In Table III are listed representative examples of specific compounds which are suitable for the purposes of this invention, when used alone in a Watt's type nickel bath or in combination with organic sulfonamides, sulfonimides and sulfonic acids of Table II.

Table III

| Compound No. | Unsaturated amides                                                   | Optimum conc., grams/liter |
|--------------|----------------------------------------------------------------------|----------------------------|
| 1            | Acrylamide                                                           | 0.1-1.2                    |
| 2            | N-acetyl acrylamide                                                  | 0.1-1.2                    |
| 3            | Cinnamic amide                                                       | 0.1-1.2                    |
| 4            | o-Chlorocinnamic amide                                               | 0.1-1.2                    |
| 5            | $\beta$ -Chloroacrylamide                                            | 0.1-1.2                    |
| 6            | 2-furanacrylamide                                                    | 0.1-1.2                    |
| 7            | p-Methoxycinnamic amide                                              | 0.1-1.2                    |
| 8            | Methacrylamide                                                       | 0.1-1.2                    |
| 9            | N-acetyl acrylamide                                                  | 0.1-1.2                    |
| 10           | Fumaramide (di-amide)                                                | 0.1-1.2                    |
| 11           | Chlorofumaramide                                                     | 0.1-1.2                    |
| 12           | Chloromaleicamide                                                    | 0.1-1.2                    |
| 13           | Maleic imide                                                         | 0.1-1.2                    |
| 14           | Phenyl maleic imide                                                  | 0.1-1.2                    |
| 15           | N-phenyl maleic imide                                                | 0.1-1.2                    |
| 16           | $\alpha$ , $\beta$ , Di-phenyl maleic imide                          | 0.1-1.2                    |
| 17           | $\alpha$ , $\beta$ , Di-phenyl maleic amide (di-amide)               | 0.1-1.2                    |
| 18           | N-nicotinoyl acrylamide                                              | 0.1-1.2                    |
| 19           | N-allyl acrylamide                                                   | 0.1-1.2                    |
| 20           | N-methyl acrylamide                                                  | 0.1-1.2                    |
| 21           | N-benzoyl acrylamide                                                 | 0.1-1.2                    |
| 22           | Atropyl amide                                                        | 0.1-1.2                    |
| 23           | Mucochloric acid amide                                               | 0.1-1.2                    |
| 24           | Mucobromic acid amide                                                | 0.1-1.2                    |
| 25           | N-tertiary Butylacrylamide                                           | 0.1-1.2                    |
| 26           | N-acrylourrea                                                        | 0.1-1.2                    |
| 27           | $\beta$ -Piperonylacrylamide                                         | 0.1-1.2                    |
| 28           | o-Hydroxy cinnamic amide                                             | 0.1-1.2                    |
| 29           | o-Methoxy cinnamic amide                                             | 0.1-1.2                    |
| 30           | p-Carbonyl-amide cinnamic amide (p-Carbonyl-amide phenyl acrylamide) | 0.1-1.2                    |
| 31           | o-Acetyl cinnamic amide                                              | 0.1-1.2                    |
| 32           | Mono 2-methoxyethyl maleic acid monoamide                            | 0.1-1.2                    |
| 33           | Allyl urea                                                           | 0.1-0.6                    |
| 34           | N-Methylol acrylamide                                                | 0.1-1.2                    |
| 35           | N-N' methylene bis-acrylamide                                        | 0.1-1.2                    |

Concentrations of allyl urea greater than 0.6 grams/liter can be used, and in combination with benzene sulfonamides and/or benzene sulfonimides when greater brightness is desired concentrations of allyl urea up to about 2 grams/liter are satisfactory, although as 2 grams/liter is approached, ductility decreases slightly.

Although Table III shows the optimum concentration of the compounds therein listed to be between 0.1 and 1.2 grams/liter, these compounds may be used in concentrations up to saturation, especially when used in conjunction with benzene sulfonamides, toluene sulfonamides and o-benzoyl sulfimide. In general, a concentration higher than about 2.5 grams/liter is unnecessary.

It will be understood that any of the compounds listed in Table III may be used separately in a Watt's type nickel bath or in combination with any of the organic sulfonamides, sulfonimides or sulfonic acids of Table II in any of the typical baths set forth in Table I. For purposes of further illustration, the examples given below set forth certain preferred embodiments of the invention.

## EXAMPLE I

|                                      | Grams/liter |
|--------------------------------------|-------------|
| NiSO <sub>4</sub> .6H <sub>2</sub> O | 250-300     |
| NiCl <sub>2</sub> .6H <sub>2</sub> O | 60          |
| H <sub>3</sub> BO <sub>3</sub>       | 45          |
| Acrylamide                           | 1.0-1.8     |
| Benzene sulfonamide                  | 0.5-3       |

## EXAMPLE II

|                                      | Grams/liter |
|--------------------------------------|-------------|
| NiSO <sub>4</sub> .6H <sub>2</sub> O | 250-300     |
| NiCl <sub>2</sub> .6H <sub>2</sub> O | 40-60       |
| H <sub>3</sub> BO <sub>3</sub>       | 40-50       |
| Cinnamic amide                       | 0.6-1.2     |
| Benzene sulfonamide                  | 0.5-3       |

## EXAMPLE III

|                                           | Grams/liter |
|-------------------------------------------|-------------|
| NiSO <sub>4</sub> .6H <sub>2</sub> O      | 50          |
| NiCl <sub>2</sub> .6H <sub>2</sub> O      | 250         |
| H <sub>3</sub> BO <sub>3</sub>            | 40-50       |
| 2-furanacrylamide                         | 0.8         |
| $\alpha$ -Benzoyl sulfimide               | 1-2         |
| $\alpha$ - or $\rho$ -Toluene sulfonamide | 1-3         |

## EXAMPLE IV

|                                   | Grams/liter |
|-----------------------------------|-------------|
| Ni(BF <sub>4</sub> ) <sub>2</sub> | 100-200     |
| H <sub>3</sub> BO <sub>3</sub>    | 30          |
| Fumaramide                        | 0.8-1.5     |
| $\alpha$ -Benzoyl sulfimide       | 1-2         |

1 Saturation.

## EXAMPLE V

|                                      | grams/liter |
|--------------------------------------|-------------|
| NiSO <sub>4</sub> .6H <sub>2</sub> O | 250         |
| NiCl <sub>2</sub> .6H <sub>2</sub> O | 35-75       |
| H <sub>3</sub> BO <sub>3</sub>       | 35-40       |
| $\alpha$ -Benzoyl sulfimide          | 0.1-2       |
| Allyl urea                           | 0.1-0.6     |
| Temperature                          | 40-65 ° C   |
| pH                                   | 2.5-4.5     |

## EXAMPLE VI

|                                      | grams/liter |
|--------------------------------------|-------------|
| NiSO <sub>4</sub> .6H <sub>2</sub> O | 250         |
| NiCl <sub>2</sub> .6H <sub>2</sub> O | 35-75       |
| H <sub>3</sub> BO <sub>3</sub>       | 35-40       |
| $\alpha$ -Benzoyl sulfimide          | 0.1-2       |
| N-Methylol acrylamide                | 0.1-1.2     |
| Temperature                          | 40-65 ° C   |
| pH                                   | 2.5-4.5     |

## EXAMPLE VII

|                                      | grams/liter |
|--------------------------------------|-------------|
| NiSO <sub>4</sub> .6H <sub>2</sub> O | 250         |
| NiCl <sub>2</sub> .6H <sub>2</sub> O | 35-75       |
| H <sub>3</sub> BO <sub>3</sub>       | 35-40       |
| $\alpha$ -Benzoyl sulfimide          | 0.1-2       |
| N-N' methylene bis-acrylamide        | 0.1-1.2     |
| Temperature                          | 40-65 ° C   |
| pH                                   | 2.5-4.5     |

The addition agents of this invention may consist of a compound or mixture of compounds represented by Formula A as such, or may consist of an admixture of at least one compound represented by Formula A and at least one compound selected from the group consisting of organic sulfonamides, sulfonimides and sulfonic acids.

This application is a continuation-in-part of my co-pending application, Serial No. 374,418, filed August 14, 1953. Serial No. 374,418 is a continuation-in-part of Serial No. 749,344, filed May 20, 1947, which is now abandoned. Application Serial No. 749,344 is a continuation-in-part of application Serial No. 366,385, filed November 20, 1940, and the present application is in part a substitute for application Serial No. 366,385, which is now abandoned.

What is claimed is:

1. A bath for electrodepositing ductile bright nickel plate comprising an aqueous acidic nickel solution consisting essentially of a material selected from the group consisting of nickel sulfate, nickel chloride, and a mixture of nickel sulfate and nickel chloride, having dissolved therein at least one compound selected from the group consisting of benzene sulfonamides and benzene sulfonimides in combination with an amount sufficient to enhance brightness of allyl urea.
2. A bath for electrodepositing ductile bright nickel plate comprising an aqueous acidic nickel solution consisting essentially of a material selected from the group consisting of nickel sulfate, nickel chloride and a mixture of nickel sulfate and nickel chloride, having dissolved therein at least one compound selected from the group consisting of benzene sulfonamides and benzene sulfonimides in combination with about 0.1 to about 0.6 gram/liter of allyl urea.
3. A method for electrodepositing ductile bright nickel

which comprises electrodepositing nickel from an aqueous acidic nickel solution consisting essentially of a material selected from the group consisting of nickel sulfate, nickel chloride and a mixture of nickel sulfate and nickel chloride having dissolved therein at least one compound selected from the group consisting of benzene sulfonamides and benzene sulfonimides in combination with an amount sufficient to enhance brightness of allyl urea.

4. A method for electrodepositing ductile bright nickel which comprises electrodepositing nickel from an aqueous

5

10

acidic nickel solution consisting essentially of a material selected from the group consisting of nickel sulfate, nickel chloride and a mixture of nickel sulfate and nickel chloride, having dissolved therein at least one compound selected from the group consisting of benzene sulfonamides and benzene sulfonimides in combination with about 0.1 to about 0.6 gram/liter of allyl urea.

**References Cited in the file of this patent**

Raub et al.: Metal Finishing, June 1940, pages 315-316.